

## UNITED STATES PATENT OFFICE

HARRY P. BASSETT, OF CYNTHIANA, KENTUCKY, AND THOMAS F. BANIGAN, OF CLIFTON HEIGHTS, PENNSYLVANIA, ASSIGNEES, BY MESNE ASSIGNMENTS, TO SAID BASSETT

## PROCESS OF MANUFACTURING ARTIFICIAL SILK AND THE LIKE

No Drawing.

Application filed May 19, 1924. Serial No. 714,497.

This invention relates to the manufacture of artificial silk, horsehair, straw, and similar films and filaments, and more particularly to the manufacture of such materials 5 from substantially pure cellulose.

It is a recognized fact in all processes for making artificial silk and similar fibres from any form of cellulose that the cellulose must be freed from all gums, resins, lignin, and 10 other non-cellulose constituents of the plant fibre from which the cellulose is obtained and the cellulose obtained essentially in a pure state. It has been found that cellulose exists in three forms, namely, the alpha, beta, and 15 gamma. Of these forms, only the alpha cellulose is useful in the preparation of artificial silk and similar fibres and films, while the beta and gamma cellulose, if present with the alpha cellulose, simply serve to dilute and injure the 20 quality of the artificial fibre without adding any additional strength.

It has been customary heretofore in purifying cellulose from plant fibres to remove the gums, resins, lignin, beta cellulose, gamma 25 cellulose and other impurities by boiling or steeping with solutions of caustic alkalies, or this procedure followed by drastic treatment with bleaching agents. In the course of our investigations, we have studied the action of 30 these treatments on various fibres such as cotton, hemp, jute, flax, etc., and have found that such treatment is injurious to the strength, purity, and yield of the resulting cellulose. Cellulose so prepared usually contains a considerable amount of beta cellulose 35 as well as decomposition products produced by the hydrolytic action of caustic alkalies employed during considerable periods of time at high temperature.

These impurities while somewhat similar to alpha cellulose in their behavior toward solvents for cellulose, when present in finished silk or similar products, act practically as inert material, thereby rendering the product 45 harsher, less uniform, weaker, and of less permanent stability than when essentially pure alpha cellulose is employed.

We have discovered that when cellulose-bearing plant fibres such as cotton, flax, hemp, 50 and ramie are subjected to a preliminary acid

treatment, in the manner described in the patent to Harry P. Bassett, granted January 3, 1922, No. 1,402,040, for a short period of time, followed by a suitable alkali boiling or steeping treatment, the resulting cellulose 55 consists essentially of pure alpha cellulose of such purity that it is suitable for the production of very high quality artificial silk, horsehair, straw, films, and similar products; and that artificial silk made from such cellulose has 60 remarkable strength, lustre, loftiness, and stability due to the absence of inert impurities. We have discovered also that by proper preliminary acid treatment followed by an alkali 65 treatment, the viscosity of the cellulose solution can be controlled between such wide limits that great flexibility is possible in the size and softness of fibres or filaments spun from a solution of such cellulose. It has been 70 possible with cellulose prepared in this manner to spin fibres ranging from one denier to 75 artificial horse-hair of 300 to 600 deniers.

It is customary in present processes for manufacture of artificial silk by the cuprammonium process to spin the silk onto rolls or 75 spools and to wash and bleach on these rolls. It is customary also to dry the silk on these or similar rolls or reels on which the silk attains essentially its complete drying. As the silk dries, it shrinks greatly, and as it is obliged 80 to dry on a rigid cylinder, the silk fibres are placed under extreme tension which is so near the elastic limit of the fibres that many of the fibres break and the texture of the silk is rendered comparatively stiff and harsh. 85

We have discovered that cuprammonium silk can be spun on rolls or reels on which the silk can be given a superficial washing to remove the main portion of the alkali and copper in the fibre, and that the silk can then 90 be removed from the roll or reel, twisted while wet, and reeled into hanks, in which form the silk can be given its final washing and bleaching treatments and can then be dried in the hank, without being held under tension, 95 to its final dryness and then wound on spools ready for use with very satisfactory results. We have found that somewhat better results can be obtained by giving the wet silk in hank form its initial drying to a moisture content 100

of 30 to 40 per cent, after which it is wound on rolls or reels and dried down to its final dryness. During this final drying, the damp silk shrinks sufficiently to develop a high lustre, somewhat better than when it is allowed to receive its entire drying in hank form without any tension.

In existing processes, it is customary to remove the last traces of copper and alkali from silk spun by the cuprammonium process by treating the wet silk with a dilute mineral acid, usually sulfuric acid. We have found that when freshly-precipitated cuprammonium filaments or films are treated with a mineral acid, particularly sulfuric acid, that it is practically impossible to remove the last traces of the mineral acid employed. These final traces of mineral acid appear to exist partly as unstable acid compounds of cellulose as, for example, cellulose sulfate. These compounds gradually decompose in the finished product, resulting in gradual deterioration of the color and strength of the finished product.

We have found that the final traces of copper and alkali can be removed from freshly-spun cuprammonium silk by organic acids, preferably acetic acid without formation of traces of acid-cellulose compounds and with no deteriorating effect on the silk. We have found that even when traces of acetic acid are left in the silk that the silk can be dried with no injurious effect.

In practicing the process forming the subject matter of the present invention, the base material used for manufacturing the silk is preferably purified cellulose, derived from plant fibres such as cotton, wood pulp, flax, hemp, ramie, etc., but we prefer to use cotton, particularly the variety known as "second-cut linters". In the preferred method, the cotton is treated as in the manner described in Patent No. 1,402,040, granted to Harry P. Bassett on January 3, 1922, by boiling with dilute acid as, for example, sulfuric acid of a strength of from 0.10 per cent to 0.24 per cent in water for about one hour, followed by boiling in dilute alkali, preferably sodium hydroxide of a strength equal to 5 to 6 pounds of alkali per 100 pounds of dry cotton for about 4 hours. The cellulose is then washed and wholly or partially freed from water.

The cellulose is then dissolved in a mixture of copper hydroxide and ammonium hydroxide. Considerable variation is possible in the proportion of copper hydroxide to cellulose but we generally use about 3 parts of copper hydroxide to 4 parts of dry cellulose, though this proportion may vary from about 1 part of copper hydroxide to 2 parts of cellulose to equal parts of each. Considerable variation can be made in the strength of ammonium hydroxide used, but in general we prefer to use ammonium hydroxide of about 20° to 26° Beaumé.

When dissolving cellulose for manufacture of artificial silk of extreme softness and finer than 80 deniers, we dissolve 4 to 6 grams of purified cellulose with 3 to 6 grams of copper hydroxide in 100 cc. of ammonium hydroxide of 20° to 26° Beaumé. When it is desired to make silk of 80 to 175 deniers, we prefer to dissolve 6 to 10 grams of purified cellulose to each 100 cc. of ammonium hydroxide.

The spinning solution so prepared is then filtered to remove particles of foreign matter and any undissolved copper compounds.

The method of spinning consists in forcing the spinning solution by low air pressure from a supply tank to the spinnerets through which it is extruded into the precipitating bath surrounding the tips of the spinnerets whereby the solution is solidified into fibres. The spinnerets may consist of a suitable number of orifices or jets arranged in small clusters to furnish a silk thread of the desired number of fibres which are together passed through a guide and from that onto a roll or reel rotating in a bath which consists of exactly or approximately the same composition as the precipitating solution. The precipitating solution may consist of a solution of sodium or potassium hydroxides or a mixture of the two, but preferably is a solution of sodium hydroxide of a concentration equivalent to 30° to 50° Beaumé. As most of the ammonia used in the spinning solution dissolves in the precipitating solution, it is necessary constantly to remove part of the solution and recover its ammonia content, replacing in the spinning bath an equal supply of fresh solution.

After a suitable amount of silk has been wound onto the roll or reel, termed the spinning cylinder, the cylinder is removed, centrifuged, or rotated rapidly for a few seconds to remove the excess of strong alkali; soaked for a few minutes in water or weak sodium hydroxide solution; is again centrifuged for a few seconds to remove most of the adhering solution; and then removed to a twisting machine. The threads are given the proper twist and are then reeled off into hanks.

In place of the stationary spinnerets, we may employ rotating spinnerets. When the silk is spun through rotating spinnerets, the subsequent twisting operation is eliminated. Otherwise, the procedure is essentially the same.

The hanks of twisted silk are slipped onto glass rods and suspended in tanks of water and washed as free as possible of copper and alkali. This operation is done by progressive extraction in a series of tanks in such a way that the copper and alkali content of the wash waters is built up so as to be economically recoverable. For example, the liquor used as the first washing of a batch of hanks may be strong enough to be sent directly to the re-

covery system, while the liquor used as the second washing for this batch of hanks may be used as the first washing liquor for the next successive batch of hanks. Or, several batches of hanks may be given their first washing in a certain liquor before it is necessary that the liquor be sent to the recovery system.

After the silk has been practically freed of soluble alkali and copper, it is soaked for a short time in a dilute solution of an organic acid, preferably acetic acid, which removes the last traces of alkali, copper, and iron.

The silk is then washed free of the last traces of copper and alkali salts by progressive washings by the same method as employed for removal of sodium hydroxide. When the acid solution containing copper and sodium acetate or sodium salt of the organic acid used is built up to an economic strength for recovery, the acid liquor is transferred to the recovery system.

If it is desired to produce bleached silk, the washed silk may next be given a bleaching treatment in an alkaline bleach of a strength not in excess of the equivalent of 6 pounds of lime bleach per 100 pounds of dry silk at a temperature not in excess of 120° F. for a short period of time, usually less than 1 hour, after which the hanks are removed from the bleach solution and immediately placed in a tank of water very slightly acidified with acetic or other organic acid, at ordinary temperature, for about 10 minutes. The hanks are then washed thoroughly in fresh water.

The hanks of silk are then hung in a dryer in which the humidity can be controlled and the silk may be gradually dried down to a moisture content of 7 per cent. It is necessary that humidity be carefully controlled during, particularly, the earlier stages of drying so that the threads on the inside and on the outside of the hank may dry essentially at the same rate. Unless this condition is controlled, there results a tendency for the threads on the outside of the hank to dry somewhat faster than the threads on the inside of the hank, producing a somewhat tangled condition in the hank.

In the preferred practice of our process, the hanks of wet silk are hung in a dryer so arranged that humidity of the atmosphere inside the drier can be accurately controlled and the silk is slowly dried to a moisture content of 30 to 40 per cent. At this point, the silk is removed, wound onto rolls or reels and returned to the drier where it is dried to a moisture content of 7 per cent. Drying in this manner allows the silk to effect its final drying under sufficient tension to bring out a high lustre, somewhat better than when it is dried directly to 7 per cent with no tension. While the tension produced on the silk fibres during drying from 30 to 40 per cent moisture to 7 per cent moisture is sufficient to develop

the full lustre of the artificial silk, this tension is insufficient to cause breaks in the fibres and, in addition, is so low that the finished silk is soft and strong.

The hanks of silk are removed from the drier, slipped onto reels and may be either rewound into hanks of any desired length or wound directly onto spools ready for use.

While we have described in detail the preferred practice of our process, it is to be understood that the details of procedure may be widely varied without departing from the spirit of the invention or the scope of the subjoined claims.

We claim:

1. In the herein described process of manufacturing artificial silk and the like, the steps of washing freshly spun cuprammonium silk filaments to remove excess alkali therefrom, twisting said filaments while in wet condition, further washing said filaments without tension, removing a major portion of the moisture content of said filaments without tension, and thereafter further reducing the moisture content of the filaments under tension.

2. In the herein described process of manufacturing artificial silk filaments and the like, the steps of partially drying wet filaments without substantial tension thereon, and thereafter further drying said filaments under tension.

3. In the herein described process of manufacturing artificial silk filaments and the like, the steps of reducing the moisture content of said filaments without tension thereon to from approximately 30 to 40 per cent moisture, and thereafter further drying said filaments under tension.

In testimony whereof, we affix our signatures.

HARRY P. BASSETT.  
THOMAS F. BANIGAN.